

Patented Oct. 1, 1929

1,730,003

## UNITED STATES PATENT OFFICE

MELVIN M. GOLDSMITH AND WILLIAM H. FALCK, OF CHICAGO, ILLINOIS; SAID FALCK  
ASSIGNOR TO GOLDSMITH BROS. SMELTING & REFINING COMPANY, A CORPORA-  
TION OF WEST VIRGINIA

### RUTHENIUM ALLOY

No Drawing.

Application filed January 3, 1927. Serial No. 158,817.

This invention relates to the manufacture of alloys of ruthenium as a substitute for the native osmiridium.

The main object is to produce a ruthenium 5 alloy having wearing qualities substantially equivalent to those of the native osmiridium. Other objects of the invention are to provide such an alloy which is easily fusible with gold; to provide such an alloy with a crystal-  
line structure so that it can be crushed into 10 small pellets such as are required for pen points; and to provide an alloy that will not crumble during grinding and slitting.

These objects are obtained by the use of 15 ruthenium in alloys in which ruthenium is the only precious metal used and in ruthenium alloys in which the ruthenium content is in excess of any other single metal of the platinum group.

20 The essential features, therefore, of the present invention are the production of alloys of ruthenium with non-precious metals such as nickel, tungsten, molybdenum, tantalum and the like; and alloys of ruthenium with 25 non-precious metals such as nickel, tungsten, molybdenum and tantalum and one or more metals of the platinum group, such as osmium, platinum, rhodium, iridium or palladium, but in which alloys the amount of ruthenium 30 shall be in excess of any other metal of the platinum group.

The alloys are produced by melting the constituents under such conditions as will insure complete fusion and a perfectly uni-  
35 form alloy, at the same time using extreme care to avoid contaminations from the refractory and from oxidation.

Illustrative alloys having the desired phys-  
ical characteristics in which ruthenium is the  
40 only metal of the platinum group present are  
successfully prepared by using ruthenium  
75%, tungsten 17½%; and nickel 7½%, or,  
ruthenium 35%, tungsten 35% and nickel  
30%. A fairly satisfactory alloy is also pre-  
45 pared by using ruthenium 15%, tungsten  
40%, nickel 32½%, tantalum 10% and mo-  
lybdenum 2½%.

And an illustrative ruthenium alloy of  
50 greater hardness is obtained when a small  
portion of osmium, palladium, rhodium,

iridium or platinum are added. Successful alloys have been prepared by using ruthenium 50%, osmium 25%, tantalum 25%, or, ruthenium 41%, osmium 40%, platinum 4½%, rhodium 1½%, tungsten 10% and 55 nickel 3%.

When the ruthenium alloy contains a member of the platinum group as given in the above illustrative alloys, the resultant alloy is harder, has better color, and takes a better 60 polish than those ruthenium alloys in which only the non-precious metals are used.

This application is a continuation in part of our copending application Serial No. 58,081, filed September 23, 1925, and contains 65 matter derived therefrom.

We claim:

1. As a substitute for osmiridium, an alloy comprising ruthenium about 75%, tungsten about 17½% and nickel about 7½%. 70
2. As a substitute for osmiridium, an alloy comprising ruthenium 75% to 35% and a complement consisting of tungsten 17% to 35%, and nickel 7½% to 30% respectively. 75

Signed at Chicago this 14th day of December, 1926.

MELVIN M. GOLDSMITH.  
WILLIAM H. FALCK.

80

85

90

95

100